

March 9, 1943.

B. F. ADAMS

2,313,114

ADHESIVE

Original Filed Nov. 8, 1937



Inventor  
Benjamin F. Adams  
by  
Walter & Kayman

Attorney

## UNITED STATES PATENT OFFICE

2,313,114

## ADHESIVE

Benjamin F. Adams, Lancaster, Pa., assignor to Armstrong Cork Company, Lancaster, Pa., a corporation of Pennsylvania

Original application November 8, 1937, Serial No. 173,407, now Patent No. 2,274,916, dated March 3, 1942. Divided and this application June 11, 1938, Serial No. 213,232

6 Claims. (Cl. 106—241)

My invention relates to an adhesive for securing hard surfaced covering materials to supporting bases. More particularly my invention relates to an adhesive for securing hard surfaced coverings which include a stratum of partible fibrous material to a supporting base, the adhesive forming a layer effective for securing the partible fibrous stratum to the base in such a manner that the floor covering may be removed from the base by rupture of the adhesive layer by reason of the effective securing properties of the adhesive being inferior to the partible qualities of the fibrous stratum.

Hard surfaced floor coverings embodying a stratum of partible material, such for example as asphalt saturated felt base having an applied paint decoration, "Linoflor," which includes a supporting stratum of asphalt saturated felt and a wear surface of oxidized oil composition, industrial flooring materials which comprise an asphalt saturated felt web having a wear surface of colored asphaltic material, "Chromalin" made in accordance with Graham and Lines Patent No. 1,971,036, including an asphalt saturated felt supporting base, and "Kolor-Flor" made in accordance with Jackson Patents Nos. 1,729,832 and 1,729,833 and Finley Patent No. 1,802,009, including a partible saturated fibrous body and, in some instances, an asphalt saturated felt carrier or base, are typical of covering materials which cannot be cemented to a supporting base and satisfactorily removed therefrom. Where a partible fibrous stratum is secured to a base by adhesive, in the manner in which linoleum is secured, for example, such coverings cannot be conveniently removed because the effective securing properties of the adhesive are greater than the partible qualities of the fibrous layer, leaving a portion of the fibrous layer attached to the floor by the adhesive.

If the partible stratum in the covering is of a waterproof type, as it is in many instances, it is important that it be removable as a whole, not only to preserve the value of the floor covering for reuse, but to facilitate the cleaning of the supporting base after such removal to receive whatever replacement covering is intended. The removal of those portions which would be disrupted from the body and attached to the floor upon attempted removal of the floor covering would be very difficult, since the binder responds to no cheap readily available solvent and, due to the waterproof binder saturating the fibrous material, the fibers are tenaciously secured to one another and present a surface in-

capable of being rendered smooth by brushing or other mechanical methods.

An object of my invention is to provide an adhesive composition effective for bonding a hard surface covering, including a stratum of partible fibrous material, to a base, the adhesive being characterized by its effective securing properties being inferior to the partible qualities of the fibrous stratum whereby the covering may be bonded directly to a supporting base and may be subsequently conveniently removed therefrom without damage to the covering and while leaving the base in condition satisfactory to receive a new covering.

Preferably, my adhesive composition is formed as follows: I place approximately 1868 pounds of alcohol (denatured) in a horizontal type mixer and add 2132 pounds of acaroid resin thereto. The mass is agitated vigorously for three hours, in which time the greater part of the acaroid resin is dissolved; a small portion of insoluble material remains in the solution. Preferably, the solution is strained to remove such insoluble material. To 3125 pounds of the strained solution, I add 1500 pounds of slate flour and thoroughly mix it therein. The composition may be placed in sealed containers until it is required for use, or it may be used immediately, as desired.

While I have described my invention with particular reference to the use of acaroid resin as an adhesive material, it will be understood other resins, either natural or synthetic, may be used in its place, for example, shellac, rosin, Manila gum, glyptal resin, or the like. Other fillers may, of course, be substituted for the slate flour in whole or in part; other vehicles may be used in place of alcohol, if desired. The above composition may be varied as desired, bearing in mind that the composition must be less resistant to tensile forces than the partible fibrous stratum which it is to secure to a base.

From experiments, I have determined certain definite limits of cohesion, within which the required feature of ready removability is obtained. I have determined that limits of cohesion of 6 to 30 pounds resistance are satisfactory. With greater tensile resistance than 30 pounds, the composition is resistant to a degree to prevent ready removability of the covering; with tensile resistance less than 6 pounds, its securing properties are dangerously weak and the covering may be loosened from the base by severe traffic and excessive wear. The "pull" test hereafter referred to as the "Scott test" used to estab-

lish these limits may be carried on in the following manner:

To one side of a strip of wood 6" long by 2" wide a thin layer of adhesive is applied, using a notched doctor blade to distribute the composition evenly over the entire surface. To the composition is immediately applied a strip of the hard surface covering 8" by 2" wide, one end of which is placed flush with one end of the strip of wood, the other end extending free beyond the wood strip. After rolling to obtain a satisfactory bond between the wood and the covering, the sample is maintained at normal room temperature for approximately four days to dry or set the adhesive. The resistance of the adhesive to tensile forces is determined by placing the sample in a Scott tensile strength machine at right angles to the direction of the forces to be exerted. The strength of the forces recorded as the covering is removed from the wood strip measures the resistance of the adhesive to tensile forces.

In the accompanying drawing illustrating my invention, there is shown a hard surface covering secured to a base, a corner of the covering being raised to show the adhesive composition effective for bonding the covering to the base. Referring to the drawing, there is shown a base 2, and a hard surface covering 3 comprising a wearing surface 4 and a stratum of particulate fibrous material 5, which may be saturated by a waterproofing compound if desired, secured to the base 2 by the adhesive composition 6. I form my building structure in the following manner: First, I prepare the base to receive a covering; that is, it is cleaned and levelled so that it presents a clean, dry, substantially smooth surface. A layer of adhesive composition is spread evenly over the base; the hard surface covering is laid thereon before the composition is dry and firmly pressed thereagainst, as by rolling, placing heavy sand bags thereover, or the like. When the adhesive composition has dried, the covering is securely attached to the base.

When it is desired to remove the covering, the adhesive composition may be readily ruptured by exerting tensile forces on the structure. When the covering is removed, the base may be readily put in condition to receive a new covering by removing the adhesive composition remaining thereon and following the process described above. I have found, in many cases, that it is not essential to remove the adhesive composition remaining on the base since a good bond may be secured by merely placing another layer thereover and securing a covering thereto. Preferably, however, I remove the adhesive composition, since, in some cases, the composition is not spread sufficiently smooth to permit a second layer thereover.

As will be apparent from the above description, my invention contemplates an adhesive which permits easy and efficient removal of the floor covering secured thereby to a base, thus obviating expensive removal costs, and eliminates the possibility of destruction of the floor covering in such removal. By the use of my adhesive, it is possible to remove the floor covering as a unit and, if the material is fit for further use, it may be relaid with facility.

This application is a division of my copending application, Serial No. 173,407, entitled Building structure, filed November 8, 1937 now Patent No. 2,274,916, dated March 3, 1942.

While I have described and illustrated a preferred embodiment of my invention, it will be understood that it is not limited to such form, since it may be otherwise embodied within the scope of the following claims.

5 I claim:

1. An adhesive composition for bonding a hard surface covering including a stratum of particulate fibrous material to a base so that the same may be removed therefrom by rupture of said adhesive without rupturing of the particulate fibrous material comprising a mixture of a solution of resin and a filler in such relative proportions that the composition when dried and solidified is rupturable within the range of from 6 to 30 pounds as determined by the "Scott test."
- 10 2. An adhesive composition for bonding a hard surface covering including a stratum of particulate fibrous material saturated with a moisture resistant substance to a base so that the same may be removed therefrom by rupture of said adhesive without rupturing of the particulate fibrous material comprising a mixture of a solution of acaroid resin and a filler in such relative proportions that the composition when dried and solidified is rupturable within the range of from 6 to 30 pounds as determined by the "Scott test."
- 15 3. An adhesive composition for bonding a hard surface covering including a stratum of particulate fibrous material saturated with a moisture resistant substance to a base so that the same may be removed therefrom by rupture of said adhesive without rupturing of the particulate fibrous material comprising a mixture of a solution of resin and filler in such relative proportions that the composition when dried and solidified is rupturable within the range of from 6 to 30 pounds as determined by the "Scott test."
- 20 4. An adhesive composition for bonding a hard surface covering including a stratum of particulate fibrous material to a base so that the same may be removed therefrom without rupturing the particulate fibrous stratum comprising a solution of acaroid resin and a filler, the proportion of resin to filler on a dry weight basis being about equal, such composition when set being resistant to tensile forces in the range of six to thirty pounds as determined by the "Scott test."
- 25 5. An adhesive composition for bonding a hard surface covering including a stratum of particulate fibrous material to a base so that the same may be removed therefrom without rupturing the particulate fibrous stratum comprising an acaroid resin solution containing about 50% of solids by weight and about an equal portion of a slate flour filler to resin solids by weight, such composition when set being resistant to tensile forces in the range of six to thirty pounds as determined by the "Scott test."
- 30 6. An adhesive composition for bonding a hard surface covering including a stratum of particulate fibrous material to a base so that the same may be removed therefrom without rupturing the particulate fibrous stratum comprising about one part by weight of acaroid resin, about one part by weight of a finely divided filler, and about one part by weight of a solvent for the acaroid resin, such composition when set being resistant to tensile forces in the range of six to thirty pounds as determined by the "Scott test."
- 35 7. An adhesive composition for bonding a hard surface covering including a stratum of particulate fibrous material to a base so that the same may be removed therefrom without rupturing the particulate fibrous stratum comprising a mixture of a solution of resin and a filler in such relative proportions that the composition when dried and solidified is rupturable within the range of from 6 to 30 pounds as determined by the "Scott test."
- 40 8. An adhesive composition for bonding a hard surface covering including a stratum of particulate fibrous material to a base so that the same may be removed therefrom without rupturing the particulate fibrous stratum comprising a solution of acaroid resin and a filler, the proportion of resin to filler on a dry weight basis being about equal, such composition when set being resistant to tensile forces in the range of six to thirty pounds as determined by the "Scott test."
- 45 9. An adhesive composition for bonding a hard surface covering including a stratum of particulate fibrous material to a base so that the same may be removed therefrom without rupturing the particulate fibrous stratum comprising a mixture of a solution of resin and a filler in such relative proportions that the composition when dried and solidified is rupturable within the range of from 6 to 30 pounds as determined by the "Scott test."
- 50 10. An adhesive composition for bonding a hard surface covering including a stratum of particulate fibrous material to a base so that the same may be removed therefrom without rupturing the particulate fibrous stratum comprising an acaroid resin solution containing about 50% of solids by weight and about an equal portion of a slate flour filler to resin solids by weight, such composition when set being resistant to tensile forces in the range of six to thirty pounds as determined by the "Scott test."
- 55 11. An adhesive composition for bonding a hard surface covering including a stratum of particulate fibrous material to a base so that the same may be removed therefrom without rupturing the particulate fibrous stratum comprising about one part by weight of acaroid resin, about one part by weight of a finely divided filler, and about one part by weight of a solvent for the acaroid resin, such composition when set being resistant to tensile forces in the range of six to thirty pounds as determined by the "Scott test."
- 60 12. An adhesive composition for bonding a hard surface covering including a stratum of particulate fibrous material to a base so that the same may be removed therefrom without rupturing the particulate fibrous stratum comprising a mixture of a solution of resin and a filler in such relative proportions that the composition when dried and solidified is rupturable within the range of from 6 to 30 pounds as determined by the "Scott test."
- 65 13. An adhesive composition for bonding a hard surface covering including a stratum of particulate fibrous material to a base so that the same may be removed therefrom without rupturing the particulate fibrous stratum comprising a solution of acaroid resin and a filler, the proportion of resin to filler on a dry weight basis being about equal, such composition when set being resistant to tensile forces in the range of six to thirty pounds as determined by the "Scott test."
- 70 14. An adhesive composition for bonding a hard surface covering including a stratum of particulate fibrous material to a base so that the same may be removed therefrom without rupturing the particulate fibrous stratum comprising a mixture of a solution of resin and a filler in such relative proportions that the composition when dried and solidified is rupturable within the range of from 6 to 30 pounds as determined by the "Scott test."

BENJAMIN F. ADAMS.